

## UNITED STATES PATENT OFFICE

2,130,996

## COPPER-ZIRCONIUM-MANGANESE ALLOY

Franz R. Hensel and Earl I. Larsen, Indianapolis, Ind., assignors to P. R. Mallory & Co., Inc., Indianapolis, Ind., a corporation of Delaware

No Drawing. Original application September 15, 1937, Serial No. 164,032. Divided and this application May 27, 1938, Serial No. 210,442

4 Claims. (CL 75—161)

This invention relates to copper alloys.

This case is a division of our co-pending application S. N. 164,032 filed September 15, 1937.

An object of the invention is to improve the characteristics of such alloys.

Other objects of the invention will be apparent from the following description taken in connection with the appended claims.

The present invention comprises the combination of elements, methods of manufacture, and the product thereof brought out and exemplified in the disclosure hereinafter set forth, the scope of the invention being indicated in the appended claims.

15 While a preferred embodiment of the invention is described herein, it is contemplated that considerable variation may be made in the method of procedure and the combination of elements without departing from the spirit of the invention.

20 The present invention relates to the improvement of alloys of copper with manganese by the addition of zirconium thereto.

According to the present invention, an alloy is made containing copper, manganese and zirconium in substantially the preferred proportions:

|           | Per cent |
|-----------|----------|
| Manganese | 0.1-5    |
| Zirconium | 0.05-5   |
| Copper    | Balance. |

It is possible, likewise, to improve the characteristics of other copper alloys containing manganese together with small percentages of additional ingredients, by the addition of zirconium.

35 For example, these alloys containing small proportions or even up to several percent of zinc, tin, calcium, lithium, magnesium, beryllium, silicon, phosphorus and silver, may be improved by the addition of zirconium in substantially the proportions indicated above.

40 Although the cost of the alloy is thereby increased we have found that for some uses, the addition of beryllium in an amount from 0.05 to 3% is particularly beneficial.

45 A preferred method of alloying is to prepare a hardener alloy, containing a high percentage of zirconium, and then introduce a predetermined amount of this alloy into a copper-manganese melt of the desired composition.

50 After the alloy has been prepared, according to such methods, a heat treatment may be carried out as follows:

The alloy in the form of a billet or a sand casting or any other form, is raised in temperature 55 to above 700° C. The alloy is then cooled quickly

(quenched) from this high temperature and subsequently aged at a temperature below 700° C.

The alloys may be cold worked after aging to further improve their characteristics. In some cases, however, it has been found advantageous 5 to introduce the cold working operation immediately after quenching and before aging.

If the alloys are subjected to a heat treatment after they have been cold worked, a phenomenon occurs which is usually called recrystallization. 10 Under certain conditions, the material might increase in grain size very considerably. Such increase in grain size will weaken the structure and the material will not flow very readily in deep drawing operations. Zirconium has been found 15 to be a most effective grain reducing element, and at the same time, being responsible for the age hardening improvements connected with the heat treatment. An example of an alloy of the present invention is:

|           | Per cent |
|-----------|----------|
| Zirconium | 1.87     |
| Manganese | 2.04     |
| Copper    | Balance. |

The maximum Rockwell B hardness after 25 straight aging is 60 Rockwell B. The electrical conductivity is 18%. If cold work is applied after quenching, and before aging, the maximum hardness can be raised to 88 Rockwell B. Cold working after complete aging will raise the hardness to 85 Rockwell B. It will be noted that the 30 electrical conductivity is very low in this case. However, for some applications, the conductivity is unimportant.

The zirconium raises the annealing temperature and at the same time provides a very fine grain structure which is particularly desirable if the material is to be worked into sheets.

The alloys of the type described are well suited 35 for use at comparatively high temperature, since hardness and electrical conductivity are maintained for indefinite periods at aging temperatures indicated.

Although the preferred proportions of manganese have been given as 0.1 to 5%, higher proportions of manganese are also permissible and come within the contemplation of this invention, namely up to 30% manganese. Manganese forms an alpha solid solution with copper throughout this range.

The most suitable range for electrical and other purposes is substantially as follows:

|           | Per cent |
|-----------|----------|
| Manganese | 1-5      |
| Zirconium | 0.5-2    |
| Copper    | Balance. |

While the present invention, as to its objects and advantages, has been described herein as carried out in specific embodiments thereof, it is not desired to be limited thereby but it is intended to cover the invention broadly within the spirit and scope of the appended claims.

What is claimed is:

1. An alloy composed of 0.05 to 5% zirconium, 0.1 to 30% manganese and the balance copper.
2. An alloy composed of 0.05 to 5% zirconium, 0.1 to 5% manganese and the balance copper.

3. An alloy composed of 0.05 to 5% zirconium, 0.1 to 5% manganese and the balance substantially all copper, characterized by high hardness and low electrical conductivity, and further characterized by the fact that its hardness and conductivity are not permanently affected by elevated temperatures.

4. An alloy composed of 0.5 to 2% zirconium, 1 to 5% manganese and the balance copper.

FRANZ R. HENSEL. 10  
EARL I. LARSEN.